



US005452755A

**United States Patent** [19]**Morikawa et al.**[11] **Patent Number:** **5,452,755**[45] **Date of Patent:** **Sep. 26, 1995**

[54] **CASTING APPARATUS FOR LOW-MELTING METALS HAVING TWO OR MORE COATING LAYERS**

5,033,721 7/1991 Gnyra ..... 266/280

**FOREIGN PATENT DOCUMENTS**

|          |        |                |         |
|----------|--------|----------------|---------|
| 1558177  | 9/1972 | Germany        | 164/418 |
| 56-6772  | 1/1981 | Japan          | .       |
| 56-68555 | 6/1981 | Japan          | 164/418 |
| 161162   | 7/1991 | Japan          | .       |
| 130675   | 1/1960 | U.S.S.R.       | 266/280 |
| 1417992  | 8/1988 | U.S.S.R.       | 266/280 |
| 2027375  | 2/1980 | United Kingdom | 164/418 |

[75] Inventors: **Katsumi Morikawa; Jyouki Yoshitomi**, both of Fukuoka, Japan

[73] Assignee: **Krosaki Corporation**, Fukuoka, Japan

[21] Appl. No.: **226,234**

[22] Filed: **Apr. 11, 1994**

**Related U.S. Application Data**

[63] Continuation of Ser. No. 955,556, Oct. 1, 1992, abandoned.

**Foreign Application Priority Data**

Oct. 9, 1991 [JP] Japan ..... 3-262358

[51] **Int. Cl.<sup>6</sup>** ..... **B22C 1/00; B22D 11/04**

[52] **U.S. Cl.** ..... **164/418; 164/138**

[58] **Field of Search** ..... 164/138, 418; 266/280, 286

**References Cited****U.S. PATENT DOCUMENTS**

|           |         |               |         |
|-----------|---------|---------------|---------|
| 4,174,972 | 11/1979 | Dreuzy et al. | 106/64  |
| 4,911,225 | 3/1990  | Leppänen      | 164/418 |
| 4,998,710 | 3/1991  | Pelton        | 266/280 |

*Primary Examiner*—Mark Rosenbaum*Assistant Examiner*—I. H. Lin*Attorney, Agent, or Firm*—Jordan and Hamburg**[57] ABSTRACT**

A casting apparatus for low-melting metals has a coating layer of two-layered structure which hardly reacts with low-melting metals, adheres firmly to the substrate, and protects the substrate from thermal and mechanical shocks for a long period of time. The layer in contact with the substrate contains glass powder having a melting point below 1000° C. and at least one binder selected from silicates and phosphates. The layer in contact with molten metal contains 5–80 wt. % of at least one fluorine compound (as a corrosion resistant material) having a melting point of above 700° C. Owing to the multiple layers, each having a specialized function, the casting apparatus has improved durability over a long period of time.

**26 Claims, 4 Drawing Sheets****10**

**FIG. 1****FIG. 2**

## FIG. 3





FIG. 4



FIG. 5



FIG. 6

**CASTING APPARATUS FOR LOW-MELTING METALS HAVING TWO OR MORE COATING LAYERS**

This application is a continuation of application Ser. No. 07/955,556 filed Oct. 1, 1992, now abandoned.

**BACKGROUND OF THE INVENTION**

1. Field of the Invention

The present invention relates to a casting apparatus having two or more coating layers, which is suitable for the casting of low-melting metals including aluminum, zinc, tin, and alloys thereof.

2. Description of the Prior Art

The casting of low-melting metals requires such apparatus as a stalk, ladle, protecting tube for the thermocouple, molten metal stirring blade, and a gas blowing tube. It is conventional practice to make these items from metal such as ferrous alloy, refractory, or ceramics.

Those apparatus which are used for the casting of aluminum alloys are usually made of, for example, cast iron, which offers high strength, low price, and good formability. Cast iron, however, has the disadvantage of being susceptible to corrosion from molten aluminum. Upon corrosion, the cast iron dissolves into the molten aluminum, which leads to contamination and deterioration of the cast aluminum.

In order to solve this problem, the use of ceramic apparatus or the coating of cast iron apparatus has been proposed.

For example, Japanese Patent Laid-open Application (KOKAI-KOHO) No. 180657/1985 discloses a ceramic stalk for low-pressure casting which is made from metallic silicon, alone or together with refractory aggregates, by nitriding sintering. The ceramic stalk prevents contamination. This merit, however, is offset by the fact that it is ten times more expensive than a cast iron stalk and that it is easily broken under load and hence has a rather short life for its high price. In addition, it is difficult to make casting apparatus of complex shapes from ceramics.

Also, Japanese Patent Laid-open No. 6772/1981 discloses the formation of a corrosion-resistant boron nitride coating on casting apparatus in contact with molten aluminum or aluminum alloy. Although boron nitride itself provides good corrosion resistance, the boron nitride coating does not provide sufficient durability because of its poor adhesion to the substrate.

A common practice to impart durability is the use of a binder. A binder for a coating on a ferrous substrate should meet the following requirements.

It does not rust the substrate during fabrication.

It should have a coefficient of thermal expansion close to that of a ferrous base metal.

It should have good adhesion to the substrate.

It should have good resistance to oxidation.

Common materials meeting these requirements are silicates and a variety of glass powders, including borosilicate glass, having a melting point below 1000° C.

There was proposed in Japanese Patent Application No. 300250/1989 [Japanese Patent Laid-open Application (KOKAI-KOHO) No. 161162/1991] a corrosion-resistant coating material containing a fluorine compound having a melting point higher than 700° C. According to the disclosure, this coating material is used to form a single coating

layer on casting apparatus for low-melting metals. However, the use of a binder is restricted by the substrate to which it is applied. Moreover, it is inconceivable that corrosion resistance varies depending on the kind of a binder.

In other words, a fluorine compound present in a single coating layer containing either an alkaline component such as silicate or a low-melting component such as borosilicate glass will undergo reduction and degrade the coating material. Therefore, the binder will not contribute to the long-term durability of the coating layer.

It is known that a coating layer does not react with low-melting metals if it contains a fluorine compound and employs a highly heat resistant binder in the form of sol such as silica sol and alumina sol. Such a coating layer, however, offers little long-term durability because its adhesion to the substrate resorts to mechanical bonding and hence, it is subject to peeling from thermal and mechanical shocks.

**SUMMARY OF THE INVENTION**

It is an object of the present invention to provide a casting apparatus for low-melting metals which has a corrosion-resistant coating layer which hardly reacts with low-melting metals, adheres firmly to the substrate, and protects the substrate from thermal and mechanical shocks for a long period of time.

**BRIEF DESCRIPTION OF THE DRAWINGS**

FIG. 1 is a sectional view showing a stalk to which the present invention is applied.

FIG. 2 is a partly cutaway perspective view showing a ladle to which the present invention is applied.

FIG. 3 is a schematic section view showing the coating layers of a multi-layered structure.

FIG. 4 is a schematic view of a stirring blade.

FIG. 5 is a schematic view of a protective tube.

FIG. 6 is a schematic view of a gas blowing tube.

**DETAILED DESCRIPTION OF THE INVENTION**

The present invention was completed on the basis of a finding that a single corrosion-resistant coating layer containing a fluorine compound is not enough to extend the life of casting apparatus for low-melting metals which depends on adhesion to the substrate, corrosion resistance, and resistance to thermal and mechanical shocks. The present invention is embodied in a casting apparatus for low-melting metals which has two or more coating layers, with the one in contact with the substrate being an adhesive coating layer containing an adhesive binder, and the one in contact with molten metal being a corrosion-resistant coating layer containing a corrosion-resistant material.

A preferred binder for the adhesive coating layer to be made on a substrate of ferrous material (such as cast iron) includes silicates (such as sodium silicate and potassium silicate) and glass powders (such as borosilicate glass) having a melting point below 1000° C. These binders may be used in combination with one another. A preferred binder for the adhesive coating layer to be made on a substrate of ceramics or refractory material includes phosphoric acid, phosphates (such as aluminum phosphate), zirconium salt, and alumina cement, in addition to the above-mentioned binders.

The binder may optionally be incorporated with one or

more fluorine compounds (such as aluminum fluoride, calcium fluoride, and magnesium fluoride) having a melting point of above 700° C. to impart corrosion resistance.

The adhesive coating layer contains refractory aggregates which include a variety of refractory oxides (such as aluminum oxide, titanium oxide, magnesium oxide, silicon oxide, zirconium oxide, chamotte, and mullite), a variety of non-oxide powders (such as silicon carbide, boron carbide, silicon nitride, boron nitride, and aluminum nitride), and metal powders which are commonly used as coating materials. The corrosion-resistant coating layer, which is in contact with molten metal, should contain one or more fluorine compounds (such as aluminum fluoride, calcium fluoride, and magnesium fluoride) having a melting point of above 700° C., in an amount of 5-80 wt. %, which impart corrosion resistance.

Examples of the binder include alumina sol, silica sol, phosphates, silane compounds, metal alkoxides, and metal acylates, which are highly heat resistant. The corrosion-resistant aggregate is selected from non-oxide powders (such as silicon carbide, boron carbide, silicon nitride, boron nitride, and aluminum nitride) and talc. It may also be selected from the above-mentioned refractory oxides to be used as the aggregate of the adhesive coating layer.

Incidentally, the binder and aggregate for the adhesive coating layer should be selected from those materials which have a coefficient of thermal expansion very close to that of the substrate.

Each layer may be formed by dipping, brushing, or spraying so that the resulting layer has a thickness of 50-200  $\mu\text{m}$ .

According to the present invention, the multi-layered coating improves the long-term durability of the substrate due to the specialized function of each layer.

The fact that the adhesive coating layer in contact with the substrate has a coefficient of thermal expansion very close to that of the substrate itself contributes to firm adhesion between the coating layer and the substrate and hence prevents the coating layer from peeling from the substrate. The adhesive coating layer formed on a ferrous substrate is especially resistant to peeling if it contains a binder selected from silicates (which are soft at low temperatures and have a comparatively high coefficient of thermal expansion) and/or a glass powder (such as borosilicate glass) having a melting point below 1000° C., because not only does it exhibit good adhesion to the substrate but it also softens at high temperatures to absorb strain. In the case of ceramic or refractory substrates, the above-mentioned binder as well as the phosphate binder produce good bonding effects, making the adhesive coating layer highly resistant to peeling.

On the other hand, the coating layer in contact with molten metal contains a fluorine compound in an amount of 5-80 wt. %, so that its surface is covered with a compact protective film which prevents the coating layer from reacting with molten metal and hence prevents the coating layer from becoming brittle.

With less than 5 wt. %, the fluorine compound (as a corrosion-resistant material) does not exhibit the desired corrosion resistance. Conversely, with an amount in excess of 80 wt. %, the fluorine compound tends to cause peeling because of an excess coefficient of thermal expansion.

If there is a big difference in the coefficient of thermal expansion between the adhesive coating layer and the corrosion resistant coating layer, it is better to interpose one or more intermediate coating layers between them, which

release the thermal stress due to the difference in thermal expansion and thus prevent one layer from peeling from the other.

## EXAMPLES

To further illustrate the invention, not by way of limitation, the following examples are given.

FIGS. 1 to 3 show some examples of the casting apparatus for low-melting metals to which the present invention can be applied.

FIG. 1 is a sectional view showing a stalk for casting which has a triple coating layer 10 formed on the surface thereof.

In FIG. 1, there is shown a substrate 1, which is the stalk proper. The coating layer 10 is composed of an adhesive coating layer 2 and a corrosion resistant coating layer 3, with an intermediate 4 layer interposed between them. The intermediate layer 4 adjusts the difference in the coefficient of thermal expansion between the two layers 2 and 3.

FIG. 2 is a partly cutaway perspective view showing a ladle which has a double coating layer 10 composed of an adhesive coating layer 2 (formed on the entire surface of the substrate 1) and a corrosion resistant layer 3 (which comes into contact with molten metal).

FIG. 3 is a schematic sectional view showing the structure of a quadruple coating layer 10 which is composed of an adhesive coating layer 2 and a corrosion resistant coating layer 3, with intermediate layers 5 and 6 interposed between them. The intermediate layer 5 has a coefficient of thermal expansion close to that of the adhesive coating layer 2, and the intermediate layer 6 has a coefficient of thermal expansion close to that of the corrosion resistant coating layer 3.

The characteristic properties of the coating layer 10 were tested in the following manner.

## TEST EXAMPLE 1

A rod having the diameter of 20 mm and the length of 100 mm was prepared as a test piece from a substrate conforming to JIS FC20 which is commonly used for casting apparatus.

The rod was provided with an adhesive coating layer 2 and a corrosion resistant coating layer 3. The former was formed from a slurry containing aggregates with a chemical composition shown in Table 1. The latter was formed from a slurry containing aggregates with a chemical composition shown in Table 2. Incidentally, the aggregates for the adhesive coating layer contain borosilicate glass powder.

TABLE 1

|                                | wt % |
|--------------------------------|------|
| Al <sub>2</sub> O <sub>3</sub> | 20   |
| SiO <sub>2</sub>               | 56   |
| MgO                            | 5    |
| Cr <sub>2</sub> O <sub>3</sub> | 4    |
| Na <sub>2</sub> O              | 4    |
| B <sub>2</sub> O <sub>3</sub>  | 9    |
| CoO                            | 2    |

TABLE 2

|     | wt % |
|-----|------|
| SiC | 55   |
| BN  | 45   |

Table 3 shows the formulations of the adhesive coating layer 2 and corrosion resistant coating layer 3, the former containing aggregates with a chemical composition shown in Table 1 and the latter containing aggregates with a chemical composition shown in Table 2. The adhesive coating layer 2 employed sodium silicate as a binder, and the corrosion resistant coating layer 3 employed silica sol as a binder. Although these binders contain water, the amounts are expressed in terms of solids because water is lost during heat treatment. The amount of water added for viscosity adjustment is indicated as an addition. Incidentally, the fluorine compound is calcium fluoride.

5

Table 3 shows the formulations of the adhesive coating layer 2 and corrosion resistant coating layer 3, the former containing aggregates with a chemical composition shown in Table 1 and the latter containing aggregates with a chemical composition shown in Table 2. The adhesive coating layer 2 employed sodium silicate as a binder, and the corrosion resistant coating layer 3 employed silica sol as a binder. Although these binders contain water, the amounts are expressed in terms of solids because water is lost during heat treatment. The amount of water added for viscosity adjustment is indicated as an addition. Incidentally, the fluorine compound is calcium fluoride.

10

Table 3 shows the formulations of the adhesive coating layer 2 and corrosion resistant coating layer 3, the former containing aggregates with a chemical composition shown in Table 1 and the latter containing aggregates with a chemical composition shown in Table 2. The adhesive coating layer 2 employed sodium silicate as a binder, and the corrosion resistant coating layer 3 employed silica sol as a binder. Although these binders contain water, the amounts are expressed in terms of solids because water is lost during heat treatment. The amount of water added for viscosity adjustment is indicated as an addition. Incidentally, the fluorine compound is calcium fluoride.

Table 3 shows the formulations of the adhesive coating layer 2 and corrosion resistant coating layer 3, the former containing aggregates with a chemical composition shown in Table 1 and the latter containing aggregates with a chemical composition shown in Table 2. The adhesive coating layer 2 employed sodium silicate as a binder, and the corrosion resistant coating layer 3 employed silica sol as a binder. Although these binders contain water, the amounts are expressed in terms of solids because water is lost during heat treatment. The amount of water added for viscosity adjustment is indicated as an addition. Incidentally, the fluorine compound is calcium fluoride.

Incidentally, the substrate has a coefficient of linear expansion of  $14.0 \times 10^{-6}/^{\circ}\text{C}$ . in the range from room temperature to  $700^{\circ}\text{C}$ .

Examples 1 to 5 show that the coating layer of double-

TABLE 3

|                                                                           | Comparative Example No. |         |         | Example No. |         |         |         |         | Comparative Example No. |         |               |
|---------------------------------------------------------------------------|-------------------------|---------|---------|-------------|---------|---------|---------|---------|-------------------------|---------|---------------|
|                                                                           | 1                       | 2       | 3       | 1           | 2       | 3       | 4       | 5       | 4                       | 5       | 6             |
| <u>Adhesive coating layer</u>                                             |                         |         |         |             |         |         |         |         |                         |         |               |
| Formulation (wt %)                                                        |                         |         |         |             |         |         |         |         |                         |         |               |
| Aggregate                                                                 | 80                      | 70      | —       | 80          | 80      | 70      | 80      | 80      | 80                      | 80      | 80            |
| Fluorine compound                                                         | 0                       | 10      | —       | 0           | 0       | 10      | 0       | 0       | 0                       | 0       | 0             |
| Sodium silicate binder (solids)                                           | 20                      | 20      | —       | 20          | 20      | 20      | 20      | 20      | 20                      | 20      | 20            |
| Water                                                                     | +40                     | +40     | —       | +40         | +40     | +40     | +40     | +40     | +40                     | +40     | +40           |
| Coefficient of thermal expansion<br>( $\times 10^{-6}/^{\circ}\text{C}$ ) | 14.0                    | 14.0    | —       | 14.0        | 14.0    | 14.5    | 14.0    | 14.0    | 14.0                    | 14.0    | 14.0          |
| Thickness of adhesive coating layer ( $\mu\text{m}$ )                     | ca. 200                 | ca. 200 | 0       | ca. 100     | ca. 100 | ca. 100 | ca. 100 | ca. 100 | ca. 100                 | ca. 100 | ca. 100       |
| Thickness of corrosion resistant coating layer ( $\mu\text{m}$ )          | 0                       | 0       | ca. 200 | ca. 100     | ca. 100 | ca. 100 | ca. 100 | ca. 100 | ca. 100                 | ca. 100 | ca. 100       |
| Adhesion of aluminum after immersion for                                  |                         |         |         |             |         |         |         |         |                         |         |               |
| 1 week                                                                    | much                    | none    | none    | none        | none    | none    | none    | none    | much                    | none    | none          |
| 4 week                                                                    | much                    | little  | none    | none        | none    | none    | none    | none    | much                    | little  | none          |
| 8 week                                                                    | much                    | none    | none    | none        | none    | none    | none    | none    | much                    | some    | none          |
| 12 week                                                                   | none                    | none    | none    | none        | none    | none    | none    | none    | none                    | much    | none          |
| After the spalling test <sup>*1</sup>                                     | intact                  | intact  | intact  | intact      | intact  | intact  | intact  | intact  | intact                  | intact  | partly peeled |
| <u>Damage to the substrate</u>                                            |                         |         |         |             |         |         |         |         |                         |         |               |
| (mm) <sup>2</sup> after                                                   |                         |         |         |             |         |         |         |         |                         |         |               |
| 1 week                                                                    | 3                       | 0       | 0       | 0           | 0       | 0       | 0       | 0       | 3                       | 0       | 0             |
| 4 week                                                                    | 18                      | 0       | 0       | 0           | 0       | 0       | 0       | 0       | 18                      | 0       | 0             |
| 8 week                                                                    | —                       | 15      | 0       | 0           | 0       | 0       | 0       | 0       | —                       | 2       | 0             |
| 12 week                                                                   | —                       | —       | 0       | 0           | 0       | 0       | 0       | 0       | —                       | 10      | 0             |

Note to Table 3

\*1 Test conditions: ( $750^{\circ}\text{C} \times 5\text{ min} \rightarrow \text{air cooling} \times 10\text{ min}$ )  $\times 20$  cycles

\*2 Damage to substrate (mm) = Diameter of substrate (20 mm) before testing -

Diameter of substrate after testing (mm)

The adhesive coating layer and corrosion resistant coating layer shown in Table 3 were formed on the substrate by brushing so that each layer was 100–200  $\mu\text{m}$  thick. After brushing, the coating layers were aged at room temperature and then heated. Some samples were prepared by brushing on the adhesive coating layer first and subsequently heating the layer, and then brushing the corrosion resistant coating layer on the adhesive coating layer and subsequently heating that.

The samples were tested after preheating by gradually immersing them in molten aluminum at  $750^{\circ}\text{C}$ . held in an alumina crucible heated in an electric furnace. After immer-

55 layer structure composed of the adhesive coating layer and the corrosion resistant coating layer (containing 5–80 wt. % fluorine compound) formed thereon remains intact for 12 weeks after immersion, with no damage to the substrate. It is also superior in spalling resistance. Presumably, this is because the adhesive coating layer functions as an adhesive to bond the corrosion resistant coating layer to the substrate while simultaneously relieving the stress which occurs between the two coating layers. In addition, Example 3 shows that the fluorine compound in the adhesive coating layer produces no adverse effect at all.

60 By contrast, Comparative Example 1 (in which the adhe-

sive coating layer contains no fluorine compound) shows that the corrosion of the substrate begins after 1 week of immersion and proceeds to such an extent that the substrate disappears almost completely after 4 weeks of immersion. Comparative Example 2 (in which the adhesive coating layer contains 10 wt. % fluorine compound) shows that the substrate remains resistant to molten aluminum for 4 weeks of immersion but disappears almost completely after 8 weeks of immersion. These results indicate that the adhesive coating layer containing sodium silicate (containing low-melting components) as a binder does not last for more than 1 month when it is used alone, even though it contains a fluorine compound. Comparative Example 3 (in which the corrosion resistant coating layer contains as much fluorine compound as in the adhesive coating layer in Comparative Example 2) shows that the substrate remains intact even after 12 weeks even though the corrosion resistance coating layer is used alone. This is attributable to the heat-resistant silica sol binder containing no low-melting components. The sample in Comparative Example 3, however, shows poor spalling resistance due to poor adhesion of the coating layer to the substrate and the difference in the coefficient of thermal expansion between the coating layer and the substrate.

Comparative Examples 4 to 6 show that even the coating layer of a double-layer structure poses a problem with durability if the content of fluorine compound in the corrosion resistant coating layer is less than 5 wt. % or more than 80 wt. %. With an amount of fluorine compound of less than 5 wt. %, the corrosion resistant coating layer is poor in corrosion resistance. With an amount of fluorine compound of more than 80 wt. %, the corrosion resistant coating layer is poor in spalling resistance due to the difference in thermal expansion between the coating layer and the substrate.

The coating layer of Example 3 was tested using an actual stalk for low-pressure casting of aluminum alloys. The stalk is made of a metal conforming to JIS FC20. The stalk with the coating layer lasted for 2.5 months without repair, whereas an ordinary stalk usually needs repair every week. In other words, the coating layer extends the life of a stalk by ten times. The test in which the coating layer pertaining to the present invention was applied to a ceramic stalk, fiber ladle, and pot crucible for melting aluminum alloys showed that it is possible to greatly reduce the amount of aluminum sticking to the casting apparatus and to greatly improve the life of the casting apparatus.

The foregoing description was made with reference to a molten aluminum alloy as a low-melting alloy. It was confirmed that the same good results as above are also obtained in the case of zinc alloys and tin alloys.

#### TEST EXAMPLE 2

The effect of an intermediate layer interposed between the adhesive coating layer and the corrosion resistant coating layer was tested. As in Test Example 1, each coating layer was made from a slurry containing an aggregate, binder, and fluorine compound in different amounts. The chemical composition of the aggregates in the adhesive coating layer is shown Table 4. The chemical composition of the aggregates in the intermediate coating layer is shown in Table 5. Incidentally, the aggregates contain borosilicate glass powder. The aggregates in the corrosion resistant coating layer have the same chemical composition as shown in Table 2.

TABLE 4

|    |                         |    | wt. % |
|----|-------------------------|----|-------|
| 5  | $\text{Al}_2\text{O}_3$ | 20 |       |
|    | $\text{SiO}_2$          | 30 |       |
|    | $\text{MgO}$            | 27 |       |
|    | $\text{Na}_2\text{O}$   | 12 |       |
| 10 | $\text{B}_2\text{O}_3$  | 9  |       |
|    | $\text{CoO}$            | 2  |       |

TABLE 5

|    |                         |    | wt. % |
|----|-------------------------|----|-------|
| 15 | $\text{Al}_2\text{O}_3$ | 23 |       |
|    | $\text{SiO}_2$          | 40 |       |
|    | $\text{MgO}$            | 20 |       |
|    | $\text{Na}_2\text{O}$   | 8  |       |
| 20 | $\text{B}_2\text{O}_3$  | 9  |       |

The adhesive coating layer and intermediate coating layer each contain sodium silicate as a binder, while the corrosion resistant coating layer contains silica sol as a binder. The fluorine compound is calcium fluoride. Although these binders contain water, their amounts are expressed in terms for solids because water is lost during heat treatment. The amount of water added for viscosity adjustment is indicated as an addition. Table 6 shows the formulation of each coating layer and the coefficient of linear expansion of the coating layer which has undergone heat treatment.

TABLE 6

|    | wt. %<br>Adhesive<br>coating<br>layer | wt. %<br>Intermediate<br>coating<br>layer | wt. %<br>Corrosion<br>resistant<br>coating<br>layer |
|----|---------------------------------------|-------------------------------------------|-----------------------------------------------------|
| 35 | 80                                    | 75                                        | 20                                                  |
| 40 | 0                                     | 5                                         | 65                                                  |
|    | 20                                    | 20                                        | 15                                                  |
|    | +40                                   | +40                                       | +85                                                 |
| 45 | 17.5                                  | 16.3                                      | 14.5                                                |

\*An average value in the range of room temperature to 700° C.

A test piece was prepared from sheet metal (SUS 304) measuring 60×120×1 mm. Incidentally, the coefficient of thermal expansion of SUS 304 is  $18.7 \times 10^{-6}/^{\circ}\text{C}$ .

The adhesive coating layer was brushed on the substrate so that a desired thickness was obtained. After brushing, the adhesive coating layer was aged at room temperature and then heated. The intermediate layer and corrosion resistant layer were brushed on the adhesive coating layer and subsequently heated so that a desired thickness was obtained. (The sample in Comparative Example 7 lacks the intermediate coating layer, and the sample in Comparative Example 8 lacks the adhesive coating layer.) The total thickness of the coating layers is 200  $\mu\text{m}$ .

For the evaluation of spalling resistance, the samples were tested after preheating by gradually immersing them in molten aluminum at 750° C. heated in an electric furnace. The molten metal is an aluminum alloy conforming to JIS ADC12. The test results are shown in Table 7.

TABLE 7

|                                               | Comparative   | Example No. |            |            | Comparative   |
|-----------------------------------------------|---------------|-------------|------------|------------|---------------|
|                                               | Example No. 7 | 6           | 7          | 8          | Example No. 8 |
| Thickness of adhesive coating layer (μm)      | ca. 100       | ca. 75      | ca. 50     | ca. 25     | 0             |
| Thickness of intermediate coating layer (μm)  | 0             | ca. 25      | ca. 50     | ca. 75     | ca. 100       |
| Thickness of corrosion resistant coating (μm) | ca. 100       | ca. 100     | ca. 100    | ca. 100    | ca. 100       |
| State after heating                           | intact        | intact      | intact     | intact     | peeled        |
| <u>Dipping spalling test</u>                  |               |             |            |            |               |
| 1st time                                      | partly peeled | no peeling  | no peeling | no peeling | (suspended)   |
| 2nd time                                      | partly peeled | no peeling  | no peeling | no peeling |               |
| 3rd time                                      | partly peeled | no peeling  | no peeling | no peeling |               |
| 4th time                                      | all peeled    | no peeling  | no peeling | no peeling |               |
| 5th time                                      | all peeled    | no peeling  | no peeling | no peeling |               |
| 10th time                                     | (suspended)   | no peeling  | no peeling | no peeling |               |
| 15th time                                     |               | no peeling  | no peeling | no peeling |               |
| 20th time                                     |               | no peeling  | no peeling | no peeling |               |

Dipping spalling test: (750° C. × 10 min. dipping → cooling at room temperature × 20 min.) × 20 cycles

Examples 6 to 8 are designed to demonstrate the effect of the intermediate coating layer interposed between the adhesive coating layer and the corrosion resistant coating layer. The intermediate layer has a coefficient of thermal expansion which is intermediately between those of the two layers. It is to be noted that the spalling resistance is greatly improved by the intermediate layer which relieves thermal stress.

By contrast, Comparative Example 7 showed poor results in which the intermediate layer is absent and the adhesive coating layer and the corrosion resistant coating layer, which greatly differ from each other in the coefficient of thermal expansion, are formed directly adjacent to each other. The coating layers remained intact after heat treatment but failed in the dipping spalling test, that is, they partly peeled in the first test and they almost completely peeled in the fourth test. Comparative Example 8 also showed poor results in which the adhesive coating layer is absent and the intermediate layer has a coefficient of thermal expansion which greatly differs from that of the substrate. The coating layers entirely peeled in the cooling cycle that followed the heating cycle due to the difference in the coefficient of thermal expansion, and hence the dipping spalling test was suspended.

FIG. 4 is a schematic view of a stirring blade A rotated by a motor B in a molten metal M in a container C. FIG. 5 is a schematic view of a protective tube showing a ladle D, a detector E for detecting the level of the molten metal M contained in the container C and a protective tube F for a thermometer. FIG. 6 is a schematic view showing an example of a gas blowing tube G blowing air and an inert gas such as Ar or N<sub>2</sub>.

The present invention has the following advantages.

- (1) It offers casting apparatus for low-melting metals, said apparatus being durable due to the adhesive coating layer and protective coating layer formed thereon which prevent the substrate from reacting with molten metal and protect the substrate from thermal and mechanical shocks.
- (2) The protective coating layer prevents the underlying adhesive coating layer from becoming brittle, and produces a secondary effect of preventing the sticking of molten metal.
- (3) The casting apparatus of improved durability dispenses with the need of frequent repairs over a long period of time.

What is claimed is:

1. A structure used in casting low-melting metals selected from the group consisting of aluminum, zinc and tin and their alloys, said structure comprising:

a substrate;

an adhesive coating layer applied by coating means selected from the group of dipping, brushing and spraying, said adhesive coating layer being in contact with said substrate, said adhesive coating layer being formed by an adhesive coating material having a melting point below 1000° C., said adhesive coating material including a first binder and a first aggregate, said first binder being selected from the group consisting of silicates, glass powder, phosphoric acid, phosphates, zirconium salt and aluminum cement, said first aggregate being selected from the group consisting of refractory oxides, non-oxide powders and metal powders, said adhesive coating layer having a thickness in the range of approximately 50 μm to 200 μm; and

a corrosion-resistant outermost coating layer applied by coating means selected from the group of dipping, brushing and spraying, said corrosion-resistant outermost coating layer contacting the molten metal carried by said casting structure, said corrosion-resistant outermost coating layer being formed by a corrosion-resistant coating material containing approximately 5-80 wt. % of at least one fluorine compound having a melting point greater than 700° C. and the remainder of said corrosive-resistant outermost coating material including a second binder and a second aggregate, said second binder being selected from the group consisting of aluminum sol, silica sol, phosphates, silane compounds, metal alkoxides and metal acylates, said second aggregate being selected from the group consisting of non-oxide powders, refractory oxides and talc, said corrosion-resistant outermost coating layer having a thickness in the range of approximately 50 μm to 200 μm.

2. A structure according to claim 1 wherein said silicates in said first binder is selected from the group consisting of sodium silicate and potassium silicate.

3. A structure according to claim 1 wherein said glass powder in said first binder is borosilicate glass.

4. A structure according to claim 1 wherein said phos-

## 11

phates in said first binder include aluminum phosphate.

5. A structure according to claim 1 wherein said refractory oxides in said first aggregate is selected from the group consisting of aluminum oxide, titanium oxide, magnesium oxide, silicon oxide, zirconium oxide, chamotte and mullite.

6. A structure according to claim 1 wherein said non-oxide powders in said first aggregate are selected from the group consisting of silicon carbide, boron carbide, silicon nitride, boron nitride, and aluminum nitride.

7. A structure according to claim 1, wherein said non-oxide powders in said second aggregate are selected from the group consisting of silicon carbide, boron carbide, silicon nitride, boron nitride, and aluminum nitride.

8. A structure according to claim 1, wherein said refractory oxides in said second aggregate are selected from the group consisting of aluminum oxide, titanium oxide, magnesium oxide, silicon oxide, zirconium oxide, chamotte and mullite.

9. A structure according to claim 1, wherein said first binder includes a fluorine compound having a melting point of about 700° C.

10. A structure according to claim 1, wherein said substrate is made of a ferrous material and said first binder is selected from silicates and glass powder.

11. A structure according to claim 1, wherein said silicates are selected from the group consisting of sodium silicates and potassium silicate and said glass powder is borosilicate glass.

12. A structure according to claim 1, wherein said substrate is made of a ceramic or a refractory material, said first binder being selected from the group consisting of phosphoric acid, phosphates, zirconium salt, and aluminum cement.

13. A structure according to claim 12, wherein said phosphates include aluminum phosphate.

14. A structure according to claim 1, wherein said fluorine compound is calcium fluoride.

15. A structure according to claim 1 wherein said corrosion-resistant coating material contains greater than 10 wt. % of said at least one fluorine compound.

16. A structure according to claim 1 wherein said adhesive coating layer is in contact with said corrosion-resistant outermost coating layer.

17. A structure according to claim 1 further comprising one or more intermediate layer between said adhesive coating layer and said corrosion-resistant outermost coating layer.

18. A structure according to claim 1, wherein said substrate has a first coefficient of thermal expansion, said adhesive coating layer having a second coefficient of thermal expansion, said corrosion-resistant outermost coating layer having a third coefficient of thermal expansion, said second coefficient of thermal expansion being intermediate said first and third coefficients of thermal expansion of said corrosive-resistant outermost layer.

19. A structure used in casting low-melting metals selected from the group consisting of aluminum, zinc and tin and their alloys, said structure comprising:

a substrate;

an adhesive coating layer in contact with the substrate and formed by an adhesive coating material having a melting point below 1000° C., said adhesive coating material including a first binder and a first aggregate, said first binder being selected from the group consisting of silicates, glass powder, phosphoric acid, phosphates, zirconium salt and aluminum cement, said first aggregate being selected from the group consisting of refractory oxides, non-oxide powders and metals powders, said adhesive coating layer having a thickness in the range of approximately 50 µm to 200 µm;

## 12

gate being selected from the group consisting of refractory oxides, non-oxide powders and metals powders, said adhesive coating layer having a thickness in the range of approximately 50 µm to 200 µm;

5 a corrosion-resistant outermost coating layer for contact with the molten metal carried by said structure, said corrosion-resistant outermost layer being formed by a corrosion-resistant coating material containing approximately 5-80 wt. % of at least one fluorine compound having a melting point greater than 700° C. and the remainder of said corrosion-resistant outermost coating material including a second binder and a second aggregate, said second binder being selected from the group consisting of aluminum sol, silica sol, phosphates, silane compounds, metal alkoxides and metal acylates, said second aggregate being selected from the group consisting of non-oxide powders, refractory oxides and talc, said corrosion-resistant outermost coating layer having a thickness in the range of approximately 50 µm to 200 µm; and

an intermediate layer between said adhesive coating layer and said corrosion-resistant outermost coating layer, said substrate, said adhesive coating layer, said intermediate layer, and said corrosion-resistant outermost coating layer having first to fourth coefficients of thermal expansion respectively, said second coefficient being less than said first coefficient said third coefficient being less than said second coefficient, and said fourth coefficient being less than said third coefficient.

15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530 9535 9540 9545 9550 9555 9560 9565 9570 9575 9580 9585 9590 9595 9600 9605 9610 9615 9620 9625 9630 9635 9640 9645 9650 9655 9660 9665 9670 9675 9680 9685 9690 9695 9700 9705 9710 9715 9720 9725 9730 9735 9740 9745 9750 9755 9760 9765 9770

**13**

rosion-resistant outermost layer being formed by a corrosion-resistant coating material containing approximately 5-80 wt. % of at least one fluorine compound having a melting point greater than 700° C. and the remainder of said corrosion-resistant outermost coating material including a second binder and a second aggregate, said second binder being selected from the group consisting of aluminum sol, silica sol, phosphates, silane compounds, metal alkoxides and metal acylates, said second aggregate being selected from the group consisting of non-oxide powders, refractory oxides and talc, said corrosion-resistant outermost coating layer having a thickness in the range of approximately 50  $\mu\text{m}$  to 200  $\mu\text{m}$ ; and

two intermediate layers positioned between said adhesive coating layer and said corrosion-resistant outermost coating layer, said two intermediate layers including an inner intermediate layer contacting said adhesive coat-

5

10

15

20

25

30

35

40

45

50

55

60

**14**

ing layer and an outer intermediate layer contacting said corrosion-resistant outermost coating layer; said substrate, said adhesive coating layer, said inner and outer intermediate layers, and said corrosion-resistant outermost coating layer each having a coefficient of thermal expansion, said coefficient of thermal expansion of said inner intermediate layering being closer to the coefficient of thermal expansion of said adhesive coating layer than to the coefficient of thermal expansion of said corrosion-resistant outermost coating layer, said coefficient of thermal expansion of said outer intermediate layer being closer to the coefficient of thermal expansion of said corrosion-resistant outermost coating layer than to the coefficient of thermal expansion of said adhesive coating layer.

\* \* \* \* \*

65